

A. JAMESON.  
ROOFING MATERIAL.

No. 73,899.

Patented Jan. 28, 1868.

Fig. 1



Fig. 2



Witnesses

W. H. Lothrop,  
S. R. T. Socie Godeur

Inventor

A. Jameson  
By his attorney  
H. C. Hanson

# United States Patent Office.

ABIEZER JAMESON, OF TRENTON, NEW JERSEY.

*Letters Patent No. 73,899, dated January 28, 1868.*

## IMPROVEMENT IN ROOFING-MATERIAL.

The Schedule referred to in these Letters Patent and making part of the same.

TO ALL WHOM IT MAY CONCERN:

Be it known that I, ABIEZER JAMESON, of Trenton, New Jersey, have invented an Improved Roofing-Material; and I do hereby declare the following to be a full, clear, and exact description of the same.

My invention consists of a sheet of paper, of the kind technically termed "felt," combined with a fabric, or with fibrous strands or filaments, as fully described hereafter, so as to form a roofing-material which is stronger and more durable than that usually employed for covering roofs, &c.

In order to enable others skilled in the art to manufacture my invention, I will now proceed to describe the manner in which the same is made, reference being had to the accompanying drawing, which forms a part of this specification, and in which—

Figure 1 represents a strip of the improved material, a portion at one corner being turned down so as to show the manner in which it is made; and

Figure 2, a section on the line 1 2, fig. 1, drawn to an enlarged scale.

The ordinary material employed for covering roofs and other surfaces, prior to applying a coating of cement, consists of strips of thick paper, technically termed "felt," which strips are nailed to the roof, and are then covered with cement.

Inasmuch as this felt possesses but little tenacity, it frequently tears or breaks when being handled, or it parts from the nails by which it is secured to the roof, thereby greatly increasing the labor and expense of covering the roofs or other surfaces. To remedy this difficulty, I combine with the "felt" a coarse textile fabric, *a*, which may be embedded in the sheet during the process of the manufacture of the latter, and while it is in a pulpy condition.

After the felt and fabric are combined, or during this operation, they may be passed through melted tar or any liquid cement, with which the felt becomes thoroughly impregnated, the material being then consolidated between presser-rollers.

Instead of textile fabric, cords or fibrous strands (formed on a card into a continuous sheet) may be embedded in the felt while in a pulpy condition. By the combination of a fibrous substance with the felt, as above described, a strong and durable material, much superior to the ordinary felt, may be manufactured at a slight expense.

I claim as my invention, and desire to secure by Letters Patent—

A roofing-material, consisting of a sheet of felt, in which is embedded a textile fabric or fibrous strands, substantially as described.

In testimony whereof, I have signed my name to this specification in the presence of two subscribing witnesses.

Witnesses:

CHARLES E. FOSTER,  
W. J. R. DELANY.

ABIEZER JAMESON.